

March 16, 1937.

L. A. SOMMER

2,074,281

METHOD AND APPARATUS FOR THE PRODUCTION OF METALLIC  
COATINGS ON ELECTRICALLY NONCONDUCTING SUBSTANCES  
BY THE THERMAL VAPORIZATION OF METALS IN VACUO

Filed July 6, 1934



Inventor:  
Ludwig A. Sommer  
by Richard E. Babcock  
Attorney

## UNITED STATES PATENT OFFICE

2,074,281

## METHOD AND APPARATUS FOR THE PRODUCTION OF METALLIC COATINGS ON ELECTRICALLY NONCONDUCTING SUBSTANCES BY THE THERMAL VAPORIZATION OF METALS IN VACUO

Ludwig August Sommer, Berlin-Dahlem,  
GermanyApplication July 6, 1934, Serial No. 734,041  
In Germany July 13, 1933

3 Claims. (Cl. 91—12.2)

The invention relates to the production of metallic coatings on electrically non-conducting substances, such as paper, textile fabrics, leather, celluloid and the like by the thermal vaporization of metals in vacuo. For this purpose vacua of  $3 \times 10^{-2}$  to about  $10^{-3}$  mm. of mercury have been employed.

I have found that in the thermal vaporization of the coating metal and the deposition of the same on electrically non-conducting materials a substantial improvement in the metallic deposits is obtained in a high vacuum.

A vacuum of say  $10^{-6}$  to  $10^{-27}$  mm. of mercury is meant as a high vacuum in this case. The deposits obtained by thermal metallic vaporization in a high vacuum on electrically non-conducting materials of all kinds, such as paper, wood, linen, wool, cotton, silk, artificial silk, jute, hemp or other textile fabrics, glass, porcelain, earthenware, leather, hides and skins, artificial masses and so forth, are distinguished by greater uniformity, greater tenacity or adhesive power, chemical purity, and freedom from oxidation, good electrical conductivity and metallic high polish.

I have further found that these coatings obtained by thermal vaporization of metals in a high vacuum are very well adapted to serve as a basis for further metallic deposits obtained electrolytically.

The invention also comprises an apparatus specially designed for carrying out the said process and which is illustrated in an example of construction in the accompanying drawing. Further features of the invention will appear from the description of the apparatus.

The drawing shows a longitudinal section of a vacuum chamber, which in the construction illustrated is formed by a section of a seamless pipe 1, both ends of which are capable of being tightly closed by covers 2 and 3. According to the invention, steel or a bronze free from pores is preferably employed as constructional material for the chamber, the walls inside, and if desired also outside, being tinned (tin coating 4). This construction has proved to be particularly advantageous in enabling the high vacuum used in the chamber to be maintained.

The evacuation of the chamber is done through 50 the pipe connection 16. On the bottom of the

chamber, a receptacle or vessel 5, consisting of insulating material or ceramic material, is arranged in known manner in the wall of which an electric resistance heater 6 is provided. The molten metal 7 is contained in the receptacle 5. 5

The web of material 8 to be metallized is slowly wound from one roller 9 on to another roller 10, and during this operation is carried past in the proximity of the opening of the receptacle 5.

According to the invention the material 8 to be metallized is strongly cooled at the place on which the metal atoms impinge. In the construction illustrated in the drawing, the cooling is effected by the guide 11 for the web of material being formed by a receptacle which projects into the 15 chamber and is partly filled with liquid air 12.

Metallic deposits which are particularly dense and adherent are obtained according to the invention by an acceleration being imparted to the vaporized metal atoms on their way from the 20 melted mass 7 to the web 8. This is effected by an electrode, for instance, an annular electrode 13, being inserted between the receptacle 5 and the material. The opposite electrode 14 is situated on the bottom of the receptacle 5. By applying 25 a high voltage, of, for example, several thousand volts, which is supplied from the source of current 15, a difference in potential is created between the melted mass 7 and the annular electrode 13, which difference of potential on the 30 positive charging of the annular electrode and negative charging of the melted metal causes a great acceleration of the vaporized negatively charged metal atoms. Consequently, the vaporized metal strikes the material to be metallized 35 with great force and metallic coatings which are particularly firmly adherent and dense are produced.

I claim:—

1. A process for producing metallic coatings 40 which consists in melting a metal, evaporating said metal under a high vacuum of about  $10^{-6}$  mm. or below of mercury, creating a potential difference between a positive electrode arranged above the surface of the metal and a negative 45 electrode connected to the metal, maintaining the said potential difference for accelerating the ions of the metal vapour and collecting the metal vapour under the said high vacuum on a surface.

2. An apparatus for producing metallic coat- 50

ings comprising a vessel, means for placing the vessel under a high vacuum, means for melting a metal, a positive electrode above the surface of the metal, a negative electrode connected to the metal, and means for applying a high potential to said electrodes.

3. An apparatus for producing metallic coatings comprising a metal vessel made of a pore free metal, a flask for containing cooling liquid,

means for feeding a surface to be metallized over the base end of the flask, means for melting a metal, a positive electrode arranged between the surface of the metal to be melted and the base end of the flask, a negative electrode connected to the metal to be melted, and means for placing the vessel under a high vacuum.

LUDWIG AUGUST SOMMER.